

## UNITED STATES PATENT OFFICE.

FREDERICK HOLBORN, OF HOBOKEN, NEW JERSEY, ASSIGNOR TO HAZELTINE CORPORATION, OF JERSEY CITY, NEW JERSEY, A CORPORATION OF DELAWARE.

## ELECTRON-EMITTING CATHODE AND PROCESS OF PREPARING THE SAME.

No Drawing.

Application filed January 14, 1926. Serial No. 81,164.

In the manufacture of oxide-coated filaments, it is necessary that the coating adhere closely to the filament and for this reason there has been extensive investigation to find 5 a suitable binder to hold the oxides on the filament. The present invention relates to the use of natural guaiac which is a resinous substance belonging to the more acid representatives of the group of resins.

10 I am aware that it has previously been suggested to use common resin, but I have found that guaiac absorbs oxygen which may be freed during the step of heating the coated filament, thereby giving the effect of 15 heating the coated filament in an oxygen atmosphere. I have further found that a large reduction in the number of coatings may be effected when a guaiac binder is used as compared with coatings in which resin is 20 used as a binder. In addition to obtaining a filament or cathode with improved emission, the cost of manufacturing is reduced by lessening the number of coatings necessary.

25 In manufacturing electron-emitting filaments with a guaiac binder commercial guaiac is refined by dissolving it in methyl-alcohol and filtering, after which the alcohol is evaporated. The refined guaiac is then 30 mixed with barium and strontium hydroxides or hydrates, or carbonates of these metals. The mixture is then ground and distilled water is added until a thick paste is formed which is applied by successively dipping the filament in the mixture or applying 35 it with a brush. The several coats are treated to reduce them to oxides.

In the event that it is desirable to employ the guaiac in solution rather than in the 40 form of paste, carbonates of the alkali-earth metals are prepared and suspended in a diluted alcohol solution of guaiac. The filament is then dipped in the solution and this operation is repeated several times in order 45 to get a plurality of coats which are then reduced to oxides by heating.

In the event that it is desired to apply the coatings in solid form, the refined guaiac is melted and carbonates are added and

stirred until the mixture solidifies. The 50 hot filament is then coated by taking a piece of the solid guaiac with the carbonates embedded therein and rubbing the solidified mixture on the hot filament until all portions of it are covered. The coating is then 55 reduced to oxides by heating.

As illustrating one way in which the method is carried out, one part of powdered refined guaiac and four parts each of strontium carbonate, barium carbonate and calcium carbonate were carefully mixed and water added so that the mixture was of such consistency that it did not drip off the filament when it was applied thereto. Ten 60 coats of this mixture were then brushed on a platinum filament ten mils wide and one-half mil thick by means of a glass-wool brush. The filament thus coated was heated in air at about 200° C. after each coat to 65 evaporate the water and guaiac, and the filament was then heated in air at about 1100° C. for one-half hour to burn down the carbonates to oxides.

I claim:

1. The process of manufacturing an electron-emitting cathode which consists in coating an electrical conductor with a compound of the alkali-earth group mixed with a material which absorbs oxygen, and then heating the coated conductor.

2. The process of manufacturing an electron-emitting cathode which consists in coating an electrical conductor with a compound of the alkali-earth group mixed with guaiac.

3. The process of manufacturing an electron-emitting cathode which consists in coating an electrical conductor with a compound of the alkali-earth group held in a guaiac binder, and then subjecting the coated filament to heat.

4. The process of manufacturing an electron-emitting cathode which consists in coating an electrical conductor with a mixture comprising a compound of the alkali-earth group and a guaiac paste, and then subjecting the coated filament to heat.

In testimony whereof I affix my signature.

FREDERICK HOLBORN.